

## UNITED STATES PATENT OFFICE

2,247,476

## MOTOR FUEL

Ulric B. Bray, Palos Verdes Estates, Calif., assignor to Union Oil Company of California, Los Angeles, Calif., a corporation of California

No Drawing. Application January 8, 1937,  
Serial No. 119,623

7 Claims. (Cl. 44—9)

This invention relates to motor fuels of the liquid type and especially motor fuels consisting primarily of cracked products such as cracked petroleum distillates.

The specific object of the invention is to add to fuels constituents derivable, at least in part, from petroleum stocks which constituents are adapted to overcome varnish and resin formations and prevent the deposition of gums and the like whereby to prevent or at least minimize the sticking of valves and rings in internal combustion engines. This applies particularly to cracked fuels which especially tend to the deposition of such gummy and resinous materials.

Primarily the invention resides in a liquid fuel, especially a cracked fuel, containing a small quantity, sufficient to overcome the above objections, of aromatic constituents of the type derived from petroleum stocks by means of selective solvents, such as the well known "Edeleanu extracts" obtained by treatment of various petroleum stocks with liquid sulfur dioxide. The invention also extends to kindred extracts obtained by other solvents or in other ways. The invention includes further the addition of a small quantity of another constituent in the form of a high boiling oxygenated gum or resin solvent of the type of dibutylphthalate, including amylphthalate, diphenyloxide, chlorodiphenyl oxide, and methyl abietate, oleate and laurate. While dibutylphthalate is preferred, with the other above mentioned solvents receiving next choice, other high boiling gum solvents may sometimes be substituted. Such possible substitution may include other high boiling esters and ethers, as well as alcohols, ketones, acids and aldehydes and kindred high boiling oxygenated gum and resin solvents. These, in turn, may contain also substituted constituents such as chlorine, sulfur, phosphorus, arsenic or selenium for the purpose of increasing oiliness or film strength where lubricated surfaces come in contact with the fuel or constituents thereof, and also for combatting corrosion. The invention also resides in a cracked or gum or resin forming fuel containing a small quantity of such a high boiling oxygenated gum solvent.

The aromatic solvent extract fractions from petroleum of the type represented by the above-mentioned "Edeleanu extracts," constitute in themselves an oil fraction of considerable lubricating value in addition to the plasticizing or softening functions which they exert upon gum, resin and varnish-type formations. Thus, the invention may be further stated as comprising

5 a motor fuel of the liquid type, such as gasoline and Diesel engine fuel, especially where the fuel is a cracked fuel, containing a small quantity of the aromatic type lubricating oil fraction adapted to soften or plasticize resin and varnish deposits, together with a small quantity of a high boiling oxygenated gum solvent of the type represented by dibutylphthalate. The small amounts to be added are in the order of 1% to 10 2% and less of the additive materials. For example about 0.3% of a mixture of one part of dibutylphthalate and two parts of an appropriate aromatic solvent-extract fraction of the type represented by liquid sulfur dioxide extracts 15 has been satisfactory in cracked gasoline. The high boiling oxygenated gum solvent serves to dissolve or loosen gums, resins and the like and the aromatic lubricating extract fraction serves to maintain all such gum and varnish deposits 20 in a plasticized condition upon or about the parts of an internal combustion engine, particularly valves, rings and fuel passages where such deposits tend to accumulate. Thus, the invention may be stated also as residing in a motor fuel 25 otherwise tending to deposit gums, resins and varnish-like materials in the fuel induction system and upon valves and rings, containing a small quantity in the order of 2%, 1% or less of an aromatic type or solvent-extract lubricating oil fraction as a plasticizer of said materials and a high boiling solvent for such materials.

In practising the present invention a suitable aromatic-type lubricating oil fraction may be obtained by any selective solvent extraction process 35 applied to petroleum stocks containing the required aromatic-type constituents. In employing such a lubricating or extract fraction, the same is preferably combined with a high boiling gum solvent. These materials may, for example, be combined in approximately equal quantities, and I have found a very desirable blend to consist of about one-third of a high boiling solvent and about two-thirds of a solvent extract from spray oil or light lubricating oil fractions such as liquid sulfur dioxide extract. These proportions, of course, may be modified so long as the required functions are obtained. This blend of the gum plasticizer and of the high boiling gum solvent is added to the gasoline, preferably only in such quantities as are necessary to overcome the resin or varnish deposits normally occurring in some types of gasoline when used in internal combustion engines. The gasolines customarily employed which tend to create such deposits are the well known cracked

gasolines and for this purpose I have found less than 1% is ordinarily adequate. For example, 0.3% produces a very satisfactory motor fuel adapted to accomplish the ends here sought. A smaller quantity may, of course, be employed with less advantageous results and likewise a larger quantity up to around 1% or 2% may be added where a particularly refractory motor fuel is concerned. The high boiling solvent preferred is dibutylphthalate and such constituent was used where 0.3% of the mixture was added to the gasoline.

With respect to the aromatic-type lubricating oil fraction a liquefied sulfur dioxide extract, commonly known as "Edeleanu extract," has been found very desirable, especially where such an extract from a spray oil stock has been mildly treated as with sulfuric acid to eliminate the more readily reactive and unsaturated constituents (as well as any tending toward a heavy or tarry nature) so as to leave a more aromatic fraction containing less reactive constituents and therefore more stable. In employing an extract of this type, it will be understood that it is preferable that the same be obtained from a stock which will yield an appropriate fraction in a suitable boiling range with respect to the gummy, resinous and varnish-like constituents which are to be controlled. For this reason, extracts from spray oil stocks are highly desirable inasmuch as they possess appropriate boiling ranges. Obviously, kindred results may be obtained with extracts of somewhat lower or higher boiling ranges, although these are often not to be preferred. For the purpose of removing the more readily reactive and more highly unsaturated constituents, a light sulfuric acid treatment may be given, for example by treating with 75 to 100 lbs. per barrel of gasoline of a 98% sulfuric acid at controlled temperatures around 100° F. but not greatly exceeding that temperature and with a limit preferably not exceeding 110° F. Preferably this acid treatment is given in two or three dumps, for example three dumps of 25 lbs. per barrel each. After separation of the sulfuric acid and contained reaction products, the remaining portion of the sulfur dioxide extract, which usually is the major portion of such extract, is neutralized with an aqueous solution of sodium hydroxide, washed with hot water, and preferably clay treated. It is then ready to be employed for the purposes of the present invention.

Again, where liquid sulfur dioxide treatment of petroleum fractions is carried on in stages, that extract from a suitable stage may be employed, for example that extract from an intermediate stage. By employing extracts from intermediate stages or from later stages of plural stage treatments, it will be possible to use extracts from heavier petroleum fractions such as from lubricating oils. This will be particularly true of extracts obtained from the treatment of light lubricating oils by various known solvent extraction methods, for example extraction by liquid sulfur dioxide and benzol mixtures. Here an intermediate or light extract may be found which will be suitable and if these extracts still contain the constituents which are too reactive, these may be further treated with an appropriate solvent, for example sulfuric acid as above described, to yield the fraction desired.

Extract fractions from petroleum stocks of the types herein indicated, including "Edeleanu extracts" are largely soluble in liquid sulfur di-

oxide, and are known to be complex mixtures of aromatic and unsaturated hydrocarbons, including alkylated naphthalenes, mono-cyclic and condensed ring compounds as well as complex sulfur and nitrogen-containing organic compounds. In addition to the aromatic or ring compounds, Edeleanu extracts also contain smaller amounts of naphthenic and paraffinic materials. They have sulfur contents ranging ordinarily from about .25% to about 3 or 4%; for example, an average kerosene extract (which might be used in some instances for the present purpose) has a sulfur content of about 1.25%, and an average spray oil extract (such as generally preferred in the present instance) may have a content of about 2.5%.

As above indicated, extracts usable here are not limited to liquid sulfur dioxide extracts but may be those obtained from other solvent extraction processes, such as those employing phenol, furfural, dichlorethyl ether, chloraniline, nitrobenzol, acetone, chlorphenol, cresylic acid and crotonaldehyde. The methods of conducting these solvent extractions and the amount of material employed are well known in the industry and need not be here described. It will be sufficient to say that around one to two volumes of solvent per volume of oil are commonly employed in countercurrent extraction and that the temperatures vary, according to the solvent, between about -10° F. and up to 125° F., being governed in part by the extent of extraction desired. For example, the average treating temperatures for liquid sulfur dioxide would be around 30° F. and for liquid sulfur dioxide-benzol mixtures around 10° F.

As above indicated, a suitable solvent extract having been segregated, the same is mixed with an equal quantity of a high boiling oxygenated gum solvent, or two or three parts of one of these agents may be employed to one part of the other and the resulting mixture blended with the gasoline tending to gum, the amount of added material being within a range of perhaps 0.1% to about 2% as may be required adequately to plasticize or to dissolve and maintain in plastic condition the gummy and varnish-like materials and prevent their accumulation in fuel induction passages and upon valves and rings to such an extent as to produce incipient sticking thereof.

The beneficial results hereof may be obtained by using extract from any light or medium viscosity lubricating oil, but I find that the more aromatic type materials, such as obtained from lighter fractions in the spray oil classification, which materials are characterized by relatively low A. P. I. gravity and high viscosity gravity constant, are preferable because of their greater efficiency and capacity to plasticize the deposits from the liquid fuels mentioned. The higher the gravity and the more paraffinic the nature, the higher will be the percentage of dibutyl phthalate or other gum solvent required. Appropriate extracts have an A. P. I. gravity range from about 10 to 20 and a viscosity of 50 to 150 seconds Saybolt Universal at 100° F.

As a specific example of a suitable extract fraction and a method of obtaining it, I have extracted a spray oil stock having a viscosity of 60 seconds Saybolt Universal at 100° F. and an A. P. I. gravity of 23.5, with liquid sulfur dioxide to yield an extract (after expulsion of the sulfur dioxide) having a gravity of 14.6 A. P. I. and a viscosity of 110 seconds at 100° F. This extract was then treated with 25 lbs. of 93%

sulfuric acid and 75 lbs. of 98% sulfuric acid per barrel at about 95° F., with a recovery of about 75%. The acid-treated extract, after neutralization had a gravity of 16.4 A. P. I., a viscosity of 80 seconds Saybolt Universal at 100° F., and a deOng number of 33. This extract was used for purposes of the present invention. The specifications for the stock, the sulfur dioxide extract, and the acid treated extract are:

|                                      | Spray<br>oil<br>stock | SO <sub>2</sub><br>extract | Acid<br>treated<br>extract |
|--------------------------------------|-----------------------|----------------------------|----------------------------|
| Saybolt viscosity at 100° F. seconds | 60                    | 110                        | 80                         |
| Gravity                              | 23.5                  | 14.6                       | 16.4                       |
| Engier distillation:                 |                       |                            |                            |
| Initial                              | °F.                   | 515                        | 530                        |
| 10%                                  | do                    | 590                        | 587                        |
| 20%                                  | do                    | 595                        | 598                        |
| 50%                                  | do                    | 625                        | 627                        |
| 90%                                  | do                    | 680                        | 684                        |
| 100%                                 | do                    | 720                        | 724                        |

While I have shown that desirable plasticizing materials are conveniently obtained by solvent extraction of petroleum oil fractions such as lubricating and spray oil stocks, similar materials, as regards both physical characteristics and plasticizing action can be obtained elsewhere, such as from certain appropriate fractions of cracking still products. For example, a cracked gas oil fraction was obtained by distillation between 575° F. and 725° F. from a cycle stock from a recycling cracking operation on a naphthenic type gas oil under liquid phase cracking conditions. Such fraction was treated with 120 lbs. 98% sulfuric acid per barrel and neutralized, and yielded a material of about 14° A. P. I. gravity with a viscosity of 75 seconds Saybolt Universal at 100° F. This extract was quite similar to the acid treated sulfur dioxide extract above described. Obviously other kindred types also may be employed.

The oxygenated gum solvents required will of course have a boiling point high enough so that they will be able to perform their desired function. Appropriate boiling points are in the general range of 550° F. or thereabouts and above at atmospheric pressure as represented by the specific materials herein mentioned.

The invention is applicable to all varieties of motor fuel tending to cause difficulty from gum deposits, and the amount of the mixture of aromatic plasticizer and high boiling gum solvent as well as the ratio of aromatic plasticizer to gum solvent is best regulated in accordance with the gum forming tendency of the gasoline. For an untreated cracked gasoline which gave 260 milligrams of gum by the well known copper dish test, 0.8% of a 75-25 mixture of dibutyl phthalate and treated spray oil extract was used. The same gasoline after treatment with one pound of 95% H<sub>2</sub>SO<sub>4</sub> per barrel and redistillation with steam gave a copper dish gum test of 90 milligrams per 100 ml. Then only 0.4% of a 75-25 mixture or 0.6% of a 50-50 mixture of dibutylphthalate and treated spray oil extract was required for successful use, or in other words, a very much smaller proportion of dibutyl phthalate. After treatment with 3 lbs. of 95% H<sub>2</sub>SO<sub>4</sub> and redistillation, the gasoline showed a copper dish gum test of 45 milligrams, and was successfully treated with 0.3% of a 2-1 mixture of spray oil extract and dibutylphthalate. Similar results are obtained with other methods of gasoline treatment prior to adding the anti-gum-

ming compounds, such as vapor phase treatment with adsorbent earth or with zinc chloride solutions.

It is observed that this invention does not constitute one of the so-called "anti-oxidant" processes where anti-oxidants are added, although it can be used in conjunction with and in addition to anti-oxidants.

It is to be understood that these disclosures are intended to be only illustrative of the generic invention, it being obvious that numerous variations not herein indicated may be developed by those skilled in the art.

I claim:

1. A motor fuel containing constituents normally tending to produce gummy and resinous deposits in internal combustion engines containing a small quantity of high boiling oxygenated gum solvent of the dibutylphthalate type together with a small quantity of a solvent extract from petroleum adapted to plasticize said gummy and resinous deposits to minimize sticking of valves and rings, said solvent extract having a gravity at least as heavy as about 16.4° A. P. I.

2. A motor fuel containing constituents otherwise tending to deposit gum and resinous materials in internal combustion engines and containing a small quantity of a mixture of a high boiling oxygenated gum solvent of the dibutylphthalate type and an aromatic extract fraction from petroleum stock free from heavy tarry and resinous and gum-forming constituents, said mixture being present in quantity adapted to plasticize said gummy and resinous constituents and to minimize the sticking of rings and valves, said extract fraction being at least as heavy as about 16.4° A. P. I.

3. A motor fuel according to claim 2 wherein solvent and plasticizing agents are added in a quantity sufficient only to avoid valve and ring sticking in internal combustion engines and the solvent is dibutylphthalate.

4. A motor fuel comprising a gasoline tending to form gums and resins, a small quantity of dibutylphthalate, and a small quantity of an aromatic extract from petroleum stock of intermediate boiling range, the dibutylphthalate and extract fraction being employed in small quantities in the order of less than about 2%.

5. A motor fuel comprising a liquid fuel containing constituents which tend to gummy and resinous deposits in internal combustion engines, a small quantity of dibutylphthalate and a small quantity of an aromatic solvent extract petroleum fraction, at least as heavy as about 16.4° A. P. I.

6. A motor fuel comprising a cracked fuel, a small quantity of dibutylphthalate and a small quantity of sulfur dioxide extract fraction from a petroleum stock of intermediate boiling range.

7. A cracked gasoline containing a small quantity of a high boiling oxygenated gum solvent of the dibutylphthalate type and a small quantity of an aromatic solvent extract fraction from petroleum stock, such fraction being largely soluble in liquid sulfur dioxide and being free from resinous and tarry constituents and from highly reactive constituents, the gum solvent and the extract fraction being employed in small quantities to minimize tendency toward valve and ring sticking in internal combustion engines, said extract fraction having a gravity between 14° and 17° A. P. I.

ULRIC B. BRAY.